# EUROPEAN PATENT SPECIFICATION

(11) **EP 2 093 314 B1**
(45) Date of publication and mention of the grant of the patent: **11.01.2017**
(21) Application number: 08161873.8
(22) Date of filing: 05.08.2008
(51) Int. Cl.: D01F 1/10

(54) **Yarns with coffee residue and preparation thereof**
Garne mit Kaffeerückständen und deren Herstellung
Fils avec des résidus de café et sa préparation

(30) Priority: 20.02.2008 TW 97105955
(43) Date of publication of application: 26.08.2009
(73) Proprietor: Magictex Apparel Corporation, Taipei Hsien 248 (TW)
(72) Inventor: Yeh, Yi-Yen, Hsinchuang City 248, Taipei Hsien (TW); Yen, Chien-Kuo, Hsinchuang City 248, Taipei Hsien (TW); Hung, Shuo-Ting, Hsinchuang City 248, Taipei Hsien (TW); Chen, Kuo-Chin, Hsinchuang City 248, Taipei Hsien (TW)
(74) Representative: Lang, Christian

(56) References cited:
- CN-A- 1 804 166
- CN-A- 101 109 122
- US-A1- 2002 037 406
- US-A1- 2005 107 505
- DATABASE WPI Week 200531 Thomson Scientific, London, GB; AN 2005-296735 XP002567398 & CN 1 558 007 A (TAIWAN PAIHO LTD) 29 December 2004 (2004-12-29)
- DATABASE WPI Week 200877 Thomson Scientific, London, GB; AN 2008-N03063 XP002567399 & CN 101 109 122 A (ZHONGLIANG IND CO LTD) 23 January 2008 (2008-01-23)

## Description

### FIELD OF THE INVENTION

The present invention relates to a preparation of yarns with coffee residue. The present invention also relates to a novel yarn with coffee residue.

### BACKGROUND

The design and development of a functional textile providing an ability of dynamic heat regulation next to the skin have attracted more and more attention in recent years. Number of attempts in this field is extensive parallel to the researches in electronics, several solar energy-based systems, buildings, etc. However, successful applications are limited and still under investigation.

It is well known that various materials such as fabrics, clothing, and other apparel can be treated to enhance the performance characteristics associated with the material. The performance characteristics can include, for example, odor adsorption, moisture control, ultra-violet light protection, and/or protection from external elements.

Certain materials naturally exhibit certain performance characteristics without being treated with chemicals or additives. For example, apparel constructed from an untreated material such as Lycra exhibits a moisture management characteristic. Materials such as Lycra; however, may not exhibit any other characteristics such as odor adsorption and/or ultraviolet protection. In addition, apparel constructed from untreated materials is limited to the physical properties (e. g., texture, feel, durability, etc.) associated with that untreated material. Moreover, the performances characteristics of such materials are often limited and do not adequately enhance the material.

After the chemicals are applied, however, the chemicals often dissipate and have to be reapplied continuously throughout the life of the fabric to impart the desired characteristics. The chemicals may dissipate, for example, when the treated fabric is washed or exposed to external elements.

It is therefore desirable to produce a high performance fabric that has desirable physical properties such as texture and durability, provides superior performance characteristics, and retains those performance characteristics after repeated use. Such a high performance fabric can be produced by treating the yarn or fiber prior to use the yarn or fiber to produce the desired material.

Approaches have been attempted to bind solid particles such as activated carbon to yarn prior to producing a fabric. Activated carbon is a granular substance that varies in size and shape depending on the process used to create the activated carbon. The activated carbon's surface area is covered with pores that also vary in size and shape depending on how it is produced. These pores provide the activated carbon with properties such as odor adsorption.

One approach involves incasing a layer of activated carbon between two layers of fabric. This technique, however, yields an odor adsorbing fabric that is heavy and cumbersome for a person to wear. Another approach that has been attempted is to incorporate the active carbon into a sheathing layer that surrounds the yarn. This approach, however, alters the physical property of yarn.

Human activity generates a great many unpleasant odors in the environment. The nature of these unpleasant odors is highly varied both on account of the physical state of the unpleasant odor particles and their chemical characteristics or their origin (biological decomposition, chemical agents, smoking, etc.). In addition, these unpleasant odors are generated in spaces or environments of everyday use such as the bathroom, kitchen, refuse, closed environments with fumes (bars), etc. In this respect, many systems have been developed to combat such unpleasant odors.

US 2005/ 0107505 A1 describes a resin composition comprising, besides other additives, coffee grounds. The resin composition can be used for molding articles including tape yarns, filaments and non-woven fabric.

### SUMMARY OF THE INVENTION

The invention is described by the method according to claim 1 and the yarn according to claim 5. Advantageous improvements of the invention are subject matter of dependent claims.

The present invention provides a method for preparing a yarn with coffee residue, comprising
(a) providing a material with coffee residue;
(b) preparing carbonized particles,
(c) preparing a mixture of the carbonized particles and the material with coffee residue, and blending said mixture with a polymer chip to produce a master batch; and
(d) drawing a yarn from the master batch added to a polymeric slurry.

The present invention also provides yarn with coffee residue, comprising a yarn and a material with coffee residue.

The present invention further provides a fabric comprising the yarn of the present invention.

### BRIEF DESCRIPTION OF THE DRAWINGS

Fig. 1 is a X1,000 Scanning Electron Microscopy (SEM) diagram of yarns with coffee residue wherein 10 represents yarn with coffee residues, 20 represents a piece of yarn and 30 represents a coffee residue.
Fig. 2 is a X2,500 SEM diagram of yarns with coffee residue, wherein 10 represents yarns with coffee residues, 20 represents a piece of yarn and 30 represents a coffee residue.
Fig. 3 is a X5,000 SEM diagram of yarns with coffee residue.

### DETAILED DESCRIPTION OF THE INVENTION

For a long time, coffee residues have been viewed as litter after the beverages coffee had been made. However, this present invention provides an environmental-friendly way to recycle the coffee residues by incorporating them into the preparation of yarns.

The present invention relates to a method for preparing a yarn with coffee residue, comprising (a) providing a mixture comprising a material with coffee residue; (b) blending the mixture with a polymer chip to produce a master batch; and (c) drawing a yarn from the master batch added to a polymeric slurry. The material with coffee residue used in the present invention is backed coffee residue, microencapsulated baked coffee residue, microencapsulated coffee essential oil, or microencapsulated fragrance organic compounds which are extracted from coffee residue. In the preferred embodiment, the coffee residue is ground coffee beans or coffee dregs. The above-mentioned mixture further comprises a carbonized particle which is prepared from carbonized coffee particle. In addition, the carbonized coffee particle is prepared by sieving coffee residue, removing organic contents from the sieved mixture, and then obtaining carbonized particles from the mixture without organic contents. Furthermore, the polymer chip in the prevent invention is selected from the group consisting of PP, Nylon or PET.

The present invention also provides a yarn, comprising a yarn and a material with coffee residue. In a preferred embodiment, the coffee residue has coffee fragrance. The material further comprises a carbonized particle. In addition this yarn can be used to make garment.

The present invention also provides a yarn with coffee fragrance, comprising a yarn which is prepared by the above-mentioned method and a material with coffee residue which has coffee fragrance. The material further comprises a carbonized particle. In addition this yarn can be used to make garment.

The present invention further provides a fabric comprising one of the above-mentioned yarns. The fabric is a non-woven fabric, a woven fabric, or a knitted fabric.

### EXAMPLES:

### EXAMPLE 1: PREPARATION OF MATERIAL WITH COFFEE RESIDUE AND CARBONIZED COFFEE PARTICLES

### 1. Preparation of material with coffee residue

The term "material with coffee residue" includes but is not limited to baked coffee residue, microencapsulated baked coffee residue; microencapsulated coffee essential oil; microencapsulated fragrance organic compounds which are extracted from coffee residue. Coffee residue could be ground coffee beans or coffee dregs in coffee shop. Then, the coffee residue was baked. Coffee essential oil could be extracted from coffee bean. The baked coffee residue or coffee essential oil was microencapsulated.

### 2. Sieving coffee residue

The coffee bean waste was rinsed in clean tap water, and then dried and ground to a particle size of 20 to 100 microns. Ground coffee beans were directly sieved. Alternatively, coffee dregs were dried and ground. Then, the ground mixture was sieved. The resulting composition can be sieved into different fine particles sizes of between 80 to 100 µm.

### 3. Removal of organic contents of sieved mixture

The sieved mixture was extracted by organic solvent to remove organic contents of the mixture. The extraction of the fat was carried out in a large Soxhlet type extractor with ethyl ether. The temperature of the extract was kept below 60°C. In all subsequent operations, air was excluded as far as possible by the use of inert gases and all solvents were freshly distilled. The lipids were treated with acetone to remove the phospholipids after which the acetone-soluble fat was recovered and saponified by refluxing with an excess of 5% alcoholic potassium hydroxide solution. The soap solution was acidified with 0.1N hydrochloric acid and the fatty acids were extracted with ether. After the fatty acids had been removed, the aqueous solution containing the water-soluble constituents was evaporated to dryness under reduced pressure and extracted with absolute alcohol for the removal of glycerol.

### 4. Preparation of carbonized particles

The mixture from step 2 was carbonized by carbonization known in the state-of-art. For example, pyrolysis is the process in which coffee mixture is heated, decomposed and eventually converted into desired product in absence of air in the fixed bed reactor. The pyrolysis includes carbonization (destructive/dry distillation of wood), charcoal processing, gasification, activated carbon processing. The pyrolysis products are wood charcoal and activated carbon. The carbonization of the coffee raw materials is done normally in the presence of chemical agents such as zinc chloride, magnesium chloride, calcium chloride or phosphoric acid. The carbonized material is treated with oxygen or noble gases in a furnace at 800-1000 °C under the conditions that permit removal of nearly all the adsorbed hydrocarbons and some of the carbon to increase the surface area.

Before subjecting the carbonized material for activation, it is washed with either acid or base depending upon the chemical used for carbonization to remove all the traces. Then it is charged for activation. Various methods are used for the activation process but the most widely used are the treatment of the carbonaceous material with oxidizing gases such as air, steam or carbon dioxide. This technique is generally used for the activation of coffee mixture, subsequent to carbonization. The charcoal is activated by reaction with steam at a temperature of 800-1100°C under controlled atmosphere in a fluidized bed reactor to facilitate uniform heat distribution and improved gas-solid contact. The reaction between steam and charcoal takes place at the internal surface area, creating more sites for adsorption with liberation of gases such as H₂, CO₂ and CO.

Initially, gasification of the carbonized material with steam occurs and the following reaction, known as the Water-Gas reaction, takes place:

C + H₂O → CO + H₂ *-175,440 kJ*/(*kg mol*)

This reaction being endothermic, temperature is maintained by partial burning of the CO and H₂ formed, as follows:

2CO + O₂ → 2CO₂ + *393,790 kJ*/(*kg mol*)

2H₂ + O2 → 2H₂O *+396,650 kJ*/(*kg mol*)*.*

### 5. Preparation of master batch

75% of the carbonized particles and 25% the material with coffee fragrance were mixed and were ground to fine particles less than 5 µm; then, the ground particles and polymer chip (such as PP, Nylon or PET) in a weight ratio of 1:9 were blended to prepare the master batch. Alternatively, 75% of the carbonized particles and 25% the material with coffee fragrance were blended into polymer chip (such as PP, Nylon or PET) to make the master batch.

### 6. Drawing yarn

The master batch was made in the industrially accepted concentrations and is added to the polymeric slurry in the same way as any other additive would be added such as for pigmentation, etc. As stated in Billie J. Collier et al., Understanding Textiles sixth edition, pressed by Prentice Hall, the master batch was designed in such a way as to allow fiber extrusion in the normal production systems. The fibers could be cut into short staple or produced in filament form and texturized, if so desired. The product yielded was a fiber that can be introduced at the blending stage of yarn production or directly into a woven or knit product so that no manufacturing processes were changed.

## Claims

1. A method for preparing a yarn with coffee residue, comprising the steps of
(a) providing a material with coffee residue,
(b) preparing carbonized coffee particles by the steps of (i) sieving coffee residue, (ii) removal of organic contents from the sieved mixture by organic solvent extraction, wherein fats are extracted, and (iii) carbonization of the mixture obtained in step (ii),
(c) preparing a mixture of the carbonized particles and the material with coffee residue, wherein said mixture is blended with a polymer chip to produce a master batch; and
(d) drawing a yarn from the master batch added to a polymeric slurry.

2. The method of claim 1, wherein the material with coffee residue is baked coffee residue, microencapsulated baked coffee residue; microencapsulated coffee essential oil; microencapsulated fragrance organic compounds which are extracted from coffee residue.

3. The method of claim 2, wherein the coffee residue is ground coffee beans or coffee dregs.

4. The method of claim 1, wherein the polymer chip is PP, Nylon or PET.

5. A yarn comprising a material with coffee residue and carbonized particles processed by the steps of (i) sieving coffee residue, (ii) removal of organic contents of the sieved mixture by organic solvent extraction, wherein fats are extracted, and (iii) carbonization of the mixture obtained in step (ii).

6. The yarn of claim 5, which is prepared by the method of claim 1.

7. A fabric comprising the yarn of claim 5.

8. The fabric of claim 7, wherein the fabric is a non-woven fabric, a woven fabric, or a knitted fabric.

9. A garment comprising the yarn of claim 5.

## Patentansprüche

1. Verfahren zur Herstellung eines Garns mit Kaffeerückständen, das die Schritte umfasst:
(a) Bereitstellen eines Materials mit Kaffeerückständen,
(b) Herstellen von karbonisierten Kaffeepartikeln durch die Schritte (i) Sieben der Kaffeerückstände, (ii) Entfernen vorn organischen Bestandteilen aus dem gesiebten Gemisch durch organische Lösungsmittelextraktion, wobei Fette extrahiert werden, und (iii) Karbonisierung des im Schritt (ii) erhaltenen Gemisches.
(c) Herstellen einer Mischung aus den karbonisierten Partikeln und dem Material mit Kaffeerückständen, wobei die besagte Mischung mit einem Kunststoffgranulat vermischt wird, um eine Grundmischung zu erzeugen, und
(d) Ziehen eines Garns aus der zu einem Polymerschlicker hinzugefügten Grundmischung.

2. Verfahren nach Anspruch 1, bei welchem das Material mit Kaffeerückständen getrocknete Kaffeerückstände, mikroverkapselte getrocknete Kaffeerückständen, mikrorrerlcapseltes ätherisches Kaffeeöl, mikroverkapselte organische Duftstoffen, die aus Kaffeerückständen extrahiert wurden, sind.

3. Verfahren nach Anspruch 2, bei welchem die Kaffeerückstände gemahlene Kaffeebohnen oder Kaffeesatz sind.

4. Verfahren nach Anspruch 1, bei welchem das Kunststoffgranulat PP, Nylon oder PET ist.

5. Garn, das ein Material mit Kaffeerückständen und karbonisierten Partikeln umfasst, die durch die Schritte (i) Sieben der Kaffeerückstände, (ii) Entfernen von organischen Bestandteilen aus dem gesiebten Gemisch durch organische Lösungsmittelextraktion, wobei Fette extrahiert werden, und (iii) Karbonisierung des im Schritt (ii) erhaltenen Gemisches, prozessiert wurden.

6. Garn nach Anspruch 5, das durch das Verfahren nach Anspruch 1 hergestellt wurde.

7. Stoff, welcher das Garn nach Anspruch 5 umfasst.

8. Stoff nach Anspruch 7, wobei der Stoff ein Vliesstoff, ein Fasergewebe oder Maschenware ist.

9. Bekleidung, welche das Garn nach Anspruch 5 umfasst.

## Revendications

1. Procédé de préparation d'un fil avec du résidu de café comprenant les étapes de
(a) fourniture d'une matière avec du résidu de café,
(b) préparation de particules de café carbonisé par les étapes de (i) tamisage du résidu de café, (ii) enlèvement du contenu organique du mélange tamisé par extraction de solvant organique, les graisses étant extraites et (iii) carbonisation du mélange obtenu à l'étape (ii),
(c) préparation d'un mélange de particules carbonisées et de la matière avec le résidu de café, ledit mélange étant mélange à un copeau de polymère pour produire un mélange-maître et
(c) extraction d'un fil du mélange-maître ajouté à une boue polymère.

2. Procédé selon la revendication 1, la matière avec le résidu de café étant du résidu de café cuit, du résidu de café cuit micro-encapsulé, de l'huile essentielle de café micro-encapsulé, des composés organiques parfumants micro-encapsulés qui sont extraits du résidu de café.

3. Procédé selon la revendication 2, le résidu de café étant des grains de café moulu ou des pastilles de café.

4. Procédé selon la revendication 1, le copeau de polymère étant du PP. du nylon ou du PET.

5. Fil comprenant une matière avec du résidu de café et des particules carbonisées traitées par les étapes de (i) tamisage du résidu de café, (ii) enlèvement du contenu organique du mélange tamisé par extraction de solvant organique, les graisses étant extraites et (iii) carbonisation du mélange obtenu à l'étape (ii).

6. Fil selon la revendication 5 qui est préparé par le procédé selon la revendication 1.

7. Tissu comprenant le fil selon la revendication 5.

8. Tissu selon la revendication 7, le tissu étant un intissé, un tissu tissé ou un tissu tricoté.

9. Vêtement comprenant le fil selon la revendication 5.
